

## UNITED STATES PATENT OFFICE

ANSEL M. KINNEY, OF CHICAGO, ILLINOIS, ASSIGNOR TO STANDARD OIL COMPANY, OF WHITING, INDIANA, A CORPORATION OF INDIANA

## TEXTILE OIL

No Drawing.

Application filed January 3, 1927. Serial No. 158,834.

The present invention relates to improvements in textile oils, and more particularly to improvements in oils intended for the preparation of rayons for use in knitting machines and in other textile machinery.

In accordance with the present invention, I prepare an oil suitable for this purpose by admixing from 90% to 50% of a purified mineral oil of low viscosity (say 50 to 60 sec. Saybolt at 100° F.) with from 1 to 20% of oleic acid and from 1 to 50% of alkali metal soaps of the sulfonic acids derived, for example, by the treatment of mineral lubricating oils with strong sulfuric acid, such as

fuming acid. With the resulting mixture I may incorporate, if desired, from 5 to 15% of a fatty oil, for example, lard oil. A preferred mixture prepared in accordance with this invention may contain about 70% of 55 sec. Saybolt (100° F.) oil; 15% of oleic acid and 15% of sodium soaps of sulfonic acids derived as above set forth. Another suitable mixture embodying the present invention is one containing 82% of mineral oil having a viscosity of 55 sec. Saybolt (100° F.); 3% of oleic acid; 10% of lard oil and 5% of sodium soaps of sulfonic compounds. As is seen from these examples, in various formulas the proportions may be widely varied and the lard oil may be employed or omitted, as desired.

In actual practice, metathesis occurs between the alkali sulfonate soaps and the oleic acid, resulting in the formation of a small amount of alkali oleate and, of course, a small amount of free sulfonic acid.

In using the oil of the present invention, it is, if necessary, diluted with a light oil to a viscosity below 70 seconds Saybolt at 100° F. (for example, cleaners' naphtha or straw oil may be used). Ordinarily very small amounts of light oil are required for this purpose; for example, with the second specific mixture above set forth, 5% of cleaners' naphtha is adequate for reducing the mixture to the desired viscosity. It is also apparent that a considerable proportion of this diluent evaporates from the treated rayon.

In preparing rayon for use in knitting machines, and particularly those of the high

speed type having rotary moving parts, it is found that the most satisfactory oil can be prepared by employing with the mineral oil the alkali metal soaps of petroleum sulfonic acids and oleic acid in approximately 55 equal proportions, their combined amount being from 20 to 40% of the entire oil.

The rayon is treated with the oil, suitably in skein form. Thus, the skeins of rayon may be immersed in a bath of the above oil 60 and subsequently centrifuged to remove excess oil, or the oil may be sprinkled upon the skeins and distributed therethrough by capillary action.

As a result of the treatment of the rayon 65 with the above oil, the fibers are softened without substantial loss in tensile strength. Fraying of the fibers is prevented, and the needles of the knitting machines upon which the rayon is used are effectively lubricated 70 and their wear reduced. Furthermore, the oil material may be readily washed from the rayon articles produced, leaving it in suitable condition for the application of such dyes as may be desired. It is found that an 75 oil of the character described is particularly effective, because it does not to any substantial degree weaken the rayons which are particularly susceptible to hydrolysis, such as those derived by the acetate process.

This application constitutes a continuation 80 in part of my application filed November 16, 1925, Serial No. 69,505.

I claim:

1. A rayon-oiling composition comprising 85 low viscosity lubricating oil, oleic acid and alkali metal soaps of oil soluble sulfonic acids derived by the treatment of mineral oils with strong sulfuric acid.

2. An oil for the treatment of rayon for 90 use in textile operations comprising from 50 to 90% of a low viscosity mineral oil, 1 to 15% of oleic acid, 1 to 50% of an alkali metal soap of an oil soluble sulfonic acid derived from the treatment of oils with sulfuric acid.

3. An oil for the treatment of rayon for 95 use in textile operations consisting of 82% of low viscosity mineral oil, 3% of oleic acid, 10% of lard oil and 5% of sodium soaps of oil soluble sulfonic acids derived 100

from the treatment of mineral oils with strong sulfuric acid.

4. An oiling composition particularly suitable for rayon-treatment comprising a low viscosity mineral oil, and approximately equal amounts of oleic acid and alkali metal soaps of oil soluble mineral oil sulfonic acids, the combined amount of said oleic acid and said soap being from 20 to 40% of the entire composition of soaps, oleic acid and oil.

5. An oil particularly suited for the treatment of rayon for use in textile operations consisting of about 70% of low viscosity mineral oil, and about 15% each of oleic acid and sodium soaps of oil soluble mineral oil sulfonic acids.

6. A rayon oiling composition comprising low viscosity mineral lubricating oil, oleic acid, fatty oil and alkali metal soaps of sulfonic oil soluble acids derived by the treatment of mineral oils with strong sulfuric acid.

7. The method of fabricating rayon cloth which comprises treating rayon fibres with a composition of low viscosity lubricating oil, oleic acid, and alkali metal soaps of oil soluble sulphonic acids derived by the treatment of mineral oils with strong sulphuric acid, and operating upon said treated fibres with machines for fabricating cloth therefrom.

8. The method of fabricating knitted rayon cloth which comprises treating rayon fibres with a composition of low viscosity lubricating oil, oleic acid, and alkali metal soaps of oil soluble sulphonic acids derived from the treatment of mineral oils with strong sulphuric acid, and operating upon said treated fibres with the needles of a knitting machine.

9. The method of fabricating rayon cloth which comprises treating rayon fibres with a composition of low viscosity purified mineral oil and alkali metal soaps of oil soluble sulphonic acids derived by the treatment of mineral oils with strong sulphuric acid, and operating upon said treated fibres with machines for fabricating cloth therefrom.

10. The composition of claim 1 wherein the lubricating oil is a purified mineral oil having a Saybolt viscosity of about 55 seconds at 100° F.

ANSEL M. KINNEY.